

Feb. 18, 1947.

A. N. OPPENHEIM

2,416,209

YARN

Filed March 12, 1946



INVENTOR  
*Austin N. Oppenheim*  
BY  
*Pauline Edmunds Morton Barron*  
ATTORNEYS

## UNITED STATES PATENT OFFICE

2,416,209

## YARN

Austin N. Oppenheim, New York, N. Y., assignor  
to Unique Fibers, Inc., New York, N. Y., a cor-  
poration of New York

Application March 12, 1946, Serial No. 653,965

5 Claims. (Cl. 37—140)

1

This invention relates to yarns made of a mixture or blend of fibres of different kinds and is concerned more particularly with a novel yarn which may be employed in the production of fabrics of unusual and attractive appearance and remarkable softness in hand and drape. The new yarn can be produced at relatively low cost for preparing and spinning operations and may be used in the manufacture of woven and knitted fabrics without changes in the machines or methods ordinarily employed.

The yarn of the invention includes a substantial proportion of animal fur, which may be either the fur or hair of animals, or a mixture of both fur and hair. Preferably, the yarn includes a mixture of furs of different characteristics, so that the fur content of the yarn may give softness, lustre, springiness, novel surface effects, etc., to fabrics made of the yarn. In addition, the yarn includes a mixture of synthetic fibres, which act as a carrier, provide body, give the yarn softness and smoothness, and also bind in the fur fibres.

In my co-pending application, Serial No. 558-464, filed October 12, 1944, I disclosed a yarn spun from a blended mixture of synthetic fibres, wool, and fur, and pointed out that the wool performed the function of binding in the other fibres and strengthening the yarn and also that the wool content gave fullness, spring, and resilience to fabrics made of the yarn. While the yarn of the co-pending application has proven highly satisfactory for many purposes, instances occur in which the presence of the wool is objectionable, because of the particular use to which fabrics made of the yarn are to be put. In my further experiments with the prior yarn, I have found that a yarn similar in its general characteristics to the prior yarn and entirely satisfactory in respect to wearing qualities and freedom from shedding of the fur fibres used, may be made by a proper selection of the constituents of the synthetic fibre content of the blended mixture to be spun.

The single figure of the drawing is a view in perspective of one form of the new yarn.

In the new yarn, I employ with the fur a mixture of synthetic fibres, which may include any of such fibres exclusive of those of organic derivatives of cellulose, that are commonly employed in yarn manufacture, together with a substantial proportion of fibres made of organic derivatives of cellulose. When such a mixture of synthetic fibres is mixed with fur and spun, the fibres of the organic derivatives of cellulose are

2

found to serve many of the useful purposes served by the wool in the prior yarn, particularly the binding function, and the new yarn may, accordingly, be employed in the production of various fabrics in which the presence of the fur content is desired but the use of wool is to be avoided.

In making the new yarn, I use animal fur of various kinds and find that mink, muskrat, wolf, squirrel, fox, beaver, ermine, nutria, opossum, sable, seal, and raccoon are most desirable. These furs differ widely in their physical characteristics and, for that reason, I prefer to use combinations of two or more different kinds of fur to obtain novel effects. For example, mink and muskrat fur may be used to advantage, because mink is soft and lustrous and gives desirable surface effects while muskrat imparts spring to the fabric. Another combination that may be used consists of opossum, which is a relatively long soft fur, and muskrat. Other desirable combinations are wolf and muskrat, fox, squirrel, and muskrat, and fox and muskrat. In general, it may be said that the short furs mainly provide characteristics of handle, drape, etc., to fabrics made of the yarn, while the long furs primarily give surface effects and provide coverage.

The blend of fibres of which the new yarn is spun is composed of fibres of synthetic materials, 30 exclusive of organic derivatives of cellulose, in amounts varying from about 10% to about 85%, fibres of organic derivatives of cellulose in amounts varying from about 10% to about 65%, and fur in amounts varying from about 10% to 35 50%. A specific example of the new yarn that is satisfactory for many purposes consists essentially of about 60% viscose rayon fibres, about 20% cellulose acetate fibres, and about 20% fur, while another form of the new yarn consists 40 essentially of about 50% viscose rayon fibres, about 25% cellulose acetate fibres, and about 20% fur. In these particular yarns, the fur content preferably includes two or more different kinds of fur, the kinds of fur being selected in view of the 45 characteristics which the yarn is to have and the nature and intended use of the fabrics into which it is to be woven or knitted.

The proportions of the constituent fibres of the yarn will vary in accordance with the characteristics, such as drape, hand, richness, softness, and appearance, that the fabrics made therefrom are to have. Also, variations in the proportions may be made in order to meet economic conditions.

The example of new yarn illustrated in the

drawing contains fibres of rayon, for example, viscose rayon, acetate fibres, relatively short fur fibres, such as mink, and longer fur fibres, such as muskrat.

In the production of the new yarn, the blended mixture of the constituents is preferably spun on the cotton system, because of the lower cost and greater ease of manufacture, and the staple lengths of the synthetic fibres used will be chosen with that end in view. Many of the fur fibres are naturally of a staple length which permits them to be handled on the cotton system, but, if the staple lengths of such fibres are too long for that purpose, the fibres may be readily shortened. It is to be understood that the new yarn can also be produced on the woolen system, in which event, fibres of longer staple length may be employed, although the cost of production of the yarn is likely to be increased.

The new yarn may be made as either a singles yarn or as a plied yarn. It will vary in count according to the type of fabric in which it is to be used and the twist will vary in the same way and also in accordance with whether it is to be used in weaving or knitting operations.

I claim:

1. A yarn which comprises a spun blended mixture containing, as essential ingredients, fibres of synthetic materials, exclusive of organic derivatives of cellulose, in an amount varying from about 10% to about 80%, fibres of organic derivatives of cellulose in an amount varying from about 10% to about 65%, and a mixture of furs of different characteristics in a total amount varying from about 10% to about 50%.

2. A yarn which comprises a spun blended mixture containing, as essential ingredients, fibres of synthetic materials, exclusive of organic

derivatives of cellulose, in an amount varying from about 10% to about 80%, fibres of organic derivatives of cellulose in an amount varying from about 10% to about 65%, and a mixture of furs of different kinds in a total amount varying from about 10% to about 50% and present, in each instance, in a substantial amount, the fibres of one kind of fur being soft and those of another kind being springy.

3. A yarn which comprises a spun blended mixture containing, as essential ingredients, fibres of synthetic materials, exclusive of organic derivatives of cellulose, in an amount varying from about 10% to about 80%, fibres of organic derivatives of cellulose in an amount varying from about 10% to about 65% and a mixture of furs of different kinds in a total amount varying from about 10% to about 50% and present, in each instance, in a substantial amount, the fibres of one kind of fur being relatively short and those of another kind being relatively long.

4. A yarn which comprises a spun blended mixture containing, as essential ingredients, about 60% of fibres of synthetic materials, exclusive of organic derivatives of cellulose, about 20% of fibres of an organic derivative of cellulose material, and about 20% of a mixture of furs of different physical characteristics.

5. A yarn which comprises a spun blended mixture containing, as essential ingredients, about 50% of fibres of synthetic materials, exclusive of organic derivatives of cellulose, about 25% of fibres of an organic derivative of cellulose material, and about 25% of a mixture of furs of different physical characteristics.

AUSTIN N. OPPENHEIM.